



US009895744B2

(12) **United States Patent**  
**Tilak et al.**

(10) **Patent No.:** **US 9,895,744 B2**  
(45) **Date of Patent:** **\*Feb. 20, 2018**

(54) **PROCESS AND APPARATUS FOR DIRECT CHILL CASTING**

(71) Applicant: **Almex USA, Inc.**, Buena Park, CA (US)

(72) Inventors: **Ravindra V. Tilak**, Orange, CA (US); **Rodney W. Wirtz**, Lake Forrest, CA (US); **Ronald M. Streigle**, Anaheim, CA (US)

(73) Assignee: **ALMEX USA, INC.**, Buena Park, CA (US)

(\*) Notice: Subject to any disclaimer, the term of this patent is extended or adjusted under 35 U.S.C. 154(b) by 507 days.

This patent is subject to a terminal disclaimer.

(21) Appl. No.: **14/401,107**

(22) PCT Filed: **May 16, 2013**

(86) PCT No.: **PCT/US2013/041459**

§ 371 (c)(1),  
(2) Date: **Nov. 13, 2014**

(87) PCT Pub. No.: **WO2013/173651**

PCT Pub. Date: **Nov. 21, 2013**

(65) **Prior Publication Data**

US 2015/0132180 A1 May 14, 2015

**Related U.S. Application Data**

(63) Continuation of application No. 13/474,614, filed on May 17, 2012, now Pat. No. 8,365,808.

(51) **Int. Cl.**

**B22D 11/049** (2006.01)  
**B22D 11/14** (2006.01)

(Continued)

(52) **U.S. Cl.**

CPC ..... **B22D 27/04** (2013.01); **B22D 7/005** (2013.01); **B22D 11/003** (2013.01);  
(Continued)

(58) **Field of Classification Search**

CPC . B22D 11/049; B22D 11/124; B22D 11/1248; B22D 11/148; B22D 11/16; B22D 11/18  
(Continued)

(56) **References Cited**

**U.S. PATENT DOCUMENTS**

|             |         |                 |
|-------------|---------|-----------------|
| 2,286,481 A | 7/1940  | Fisher          |
| 2,863,558 A | 12/1958 | Brondyke et al. |

(Continued)

**FOREIGN PATENT DOCUMENTS**

|    |         |         |
|----|---------|---------|
| CA | 1309870 | 11/1992 |
| CN | 1059484 | 3/1992  |

(Continued)

**OTHER PUBLICATIONS**

Almex USA, Inc., "International preliminary report on patentability", PCT Application No. PCT/US2013/041457, (dated Nov. 27, 2014), 7 pages.

(Continued)

*Primary Examiner* — Kevin E Yoon

(74) *Attorney, Agent, or Firm* — Womble Bond Dickinson (US) LLP

(57) **ABSTRACT**

A process in direct chill casting wherein molten metal is introduced into a casting mold and cooled by impingement of a liquid coolant on solidifying metal in a casting pit including a movable platen and an occurrence of a bleed-out or run-out is detected the process including exhausting generated gas from the casting pit; and introducing an inert gas into the casting pit, the inert gas having a density less than a density of air; reducing any flow of the liquid coolant.

**32 Claims, 3 Drawing Sheets**



|      |                                                   |                                                                                                                                                                                                                                                                         |                 |             |                     |                    |  |
|------|---------------------------------------------------|-------------------------------------------------------------------------------------------------------------------------------------------------------------------------------------------------------------------------------------------------------------------------|-----------------|-------------|---------------------|--------------------|--|
| (51) | <b>Int. Cl.</b>                                   |                                                                                                                                                                                                                                                                         |                 |             |                     |                    |  |
|      | <i>B22D 27/04</i>                                 | (2006.01)                                                                                                                                                                                                                                                               | 4,858,674 A     | 8/1989      | Enright             |                    |  |
|      | <i>B22D 11/00</i>                                 | (2006.01)                                                                                                                                                                                                                                                               | 4,930,566 A     | 6/1990      | Yanagimoto et al.   |                    |  |
|      | <i>B22D 7/00</i>                                  | (2006.01)                                                                                                                                                                                                                                                               | 4,947,925 A     | 8/1990      | Wagstaff et al.     |                    |  |
|      | <i>B22D 11/16</i>                                 | (2006.01)                                                                                                                                                                                                                                                               | 4,964,993 A     | 10/1990     | Stankiewicz         |                    |  |
|      | <i>B22D 11/18</i>                                 | (2006.01)                                                                                                                                                                                                                                                               | 4,986,337 A     | 1/1991      | Soulier             |                    |  |
|      | <i>B22D 27/00</i>                                 | (2006.01)                                                                                                                                                                                                                                                               | 4,987,950 A     | 1/1991      | Yu                  |                    |  |
|      | <i>B22D 30/00</i>                                 | (2006.01)                                                                                                                                                                                                                                                               | 5,028,570 A     | 7/1991      | Winkelbauer et al.  |                    |  |
|      | <i>B22D 46/00</i>                                 | (2006.01)                                                                                                                                                                                                                                                               | 5,032,171 A     | 7/1991      | Robare et al.       |                    |  |
|      | <i>C22C 21/00</i>                                 | (2006.01)                                                                                                                                                                                                                                                               | 5,052,469 A     | 10/1991     | Yanagimoto et al.   |                    |  |
|      |                                                   |                                                                                                                                                                                                                                                                         | 5,091,149 A     | 2/1992      | Shin et al.         |                    |  |
|      |                                                   |                                                                                                                                                                                                                                                                         | 5,148,853 A     | 9/1992      | Yu et al.           |                    |  |
|      |                                                   |                                                                                                                                                                                                                                                                         | 5,167,918 A     | 12/1992     | Shin et al.         |                    |  |
|      |                                                   |                                                                                                                                                                                                                                                                         | 5,176,197 A     | 1/1993      | Hamaguchi et al.    |                    |  |
|      |                                                   |                                                                                                                                                                                                                                                                         | 5,185,297 A     | 2/1993      | Park et al.         |                    |  |
| (52) | <b>U.S. Cl.</b>                                   |                                                                                                                                                                                                                                                                         |                 |             |                     |                    |  |
|      | CPC .....                                         | <i>B22D 11/049</i> (2013.01); <i>B22D 11/148</i> (2013.01); <i>B22D 11/16</i> (2013.01); <i>B22D 11/18</i> (2013.01); <i>B22D 27/003</i> (2013.01); <i>B22D 27/045</i> (2013.01); <i>B22D 30/00</i> (2013.01); <i>B22D 46/00</i> (2013.01); <i>C22C 21/00</i> (2013.01) | 5,212,343 A     | 5/1993      | Bruppacher et al.   |                    |  |
|      |                                                   |                                                                                                                                                                                                                                                                         | 5,320,803 A     | 6/1994      | Webster             |                    |  |
| (58) | <b>Field of Classification Search</b>             |                                                                                                                                                                                                                                                                         |                 |             |                     |                    |  |
|      | USPC ....                                         | 164/151.5, 415, 444, 452, 475, 486, 487                                                                                                                                                                                                                                 | 5,369,063 A     | 11/1994     | Gee                 |                    |  |
|      | See application file for complete search history. |                                                                                                                                                                                                                                                                         | 5,404,813 A     | 4/1995      | Wong                |                    |  |
| (56) | <b>References Cited</b>                           |                                                                                                                                                                                                                                                                         |                 |             |                     |                    |  |
|      | U.S. PATENT DOCUMENTS                             |                                                                                                                                                                                                                                                                         |                 |             |                     |                    |  |
|      | 3,006,473 A                                       | 10/1961 Gamber                                                                                                                                                                                                                                                          | 5,415,220 A     | 5/1995      | Edwards             |                    |  |
|      | 3,235,089 A                                       | 2/1966 Burroughs                                                                                                                                                                                                                                                        | 5,427,602 A     | 6/1995      | Deyoung et al.      |                    |  |
|      | 3,281,238 A                                       | 10/1966 Bachowski et al.                                                                                                                                                                                                                                                | 5,441,919 A     | 8/1995      | Park et al.         |                    |  |
|      | 3,320,348 A                                       | 5/1967 Seulen et al.                                                                                                                                                                                                                                                    | 5,548,520 A     | 8/1996      | Nakamura et al.     |                    |  |
|      | 3,335,212 A                                       | 8/1967 Seulen et al.                                                                                                                                                                                                                                                    | 5,845,481 A     | 12/1998     | Briesch et al.      |                    |  |
|      | 3,451,465 A                                       | 6/1969 Moritz et al.                                                                                                                                                                                                                                                    | 5,846,481 A     | 12/1998     | Tilak               |                    |  |
|      | 3,524,548 A                                       | 8/1970 McDonald et al.                                                                                                                                                                                                                                                  | 5,873,405 A     | 2/1999      | Carrier et al.      |                    |  |
|      | 3,800,856 A *                                     | 4/1974 Mizikar .....                                                                                                                                                                                                                                                    | 6,069,910 A     | 5/2000      | Eckert              |                    |  |
|      |                                                   | <i>B22D 11/1246</i>                                                                                                                                                                                                                                                     | 6,148,018 A     | 11/2000     | Garcia et al.       |                    |  |
|      |                                                   | 164/256                                                                                                                                                                                                                                                                 | 6,279,645 B1    | 8/2001      | McGtade et al.      |                    |  |
|      |                                                   |                                                                                                                                                                                                                                                                         | 6,393,044 B1    | 5/2002      | Fishman et al.      |                    |  |
|      |                                                   |                                                                                                                                                                                                                                                                         | 6,398,844 B1    | 6/2002      | Hobbs et al.        |                    |  |
|      |                                                   |                                                                                                                                                                                                                                                                         | 6,446,704 B1 *  | 9/2002      | Collins .....       | <i>B22D 11/148</i> |  |
|      |                                                   |                                                                                                                                                                                                                                                                         |                 |             |                     | 164/151.5          |  |
|      | 3,834,445 A                                       | 9/1974 Raschke                                                                                                                                                                                                                                                          | 6,491,087 B1    | 12/2002     | Tilak               |                    |  |
|      | 3,895,937 A                                       | 7/1975 Gjosteen et al.                                                                                                                                                                                                                                                  | 6,551,424 B1    | 4/2003      | Haszler et al.      |                    |  |
|      | 3,947,363 A                                       | 3/1976 Pryor et al.                                                                                                                                                                                                                                                     | 6,675,870 B2    | 1/2004      | Tilak               |                    |  |
|      | 4,113,241 A                                       | 9/1978 Dore                                                                                                                                                                                                                                                             | 6,808,009 B2    | 10/2004     | Anderson            |                    |  |
|      | 4,188,884 A                                       | 2/1980 White et al.                                                                                                                                                                                                                                                     | 6,837,300 B2    | 1/2005      | Cooper et al.       |                    |  |
|      | 4,214,624 A                                       | 7/1980 Foye et al.                                                                                                                                                                                                                                                      | 7,000,676 B2    | 2/2006      | Chu et al.          |                    |  |
|      | 4,221,589 A                                       | 9/1980 Verstraeten                                                                                                                                                                                                                                                      | 7,204,295 B2    | 4/2007      | Schneider et al.    |                    |  |
|      | 4,237,961 A                                       | 12/1980 Zinniger                                                                                                                                                                                                                                                        | 7,296,613 B2    | 11/2007     | Anderson et al.     |                    |  |
|      | 4,248,630 A                                       | 2/1981 Balmuth                                                                                                                                                                                                                                                          | 7,550,028 B2    | 6/2009      | Riquer et al.       |                    |  |
|      | 4,355,679 A                                       | 10/1982 Wilkins                                                                                                                                                                                                                                                         | 8,056,611 B2    | 11/2011     | Gildemeister et al. |                    |  |
|      | 4,395,333 A                                       | 7/1983 Groteke                                                                                                                                                                                                                                                          | 8,196,641 B2    | 6/2012      | Jacques et al.      |                    |  |
|      | 4,427,185 A                                       | 1/1984 Meyer                                                                                                                                                                                                                                                            | 8,365,808 B1    | 2/2013      | Tilak et al.        |                    |  |
|      | 4,444,377 A                                       | 4/1984 Groteke et al.                                                                                                                                                                                                                                                   | 8,479,802 B1    | 7/2013      | Tilak et al.        |                    |  |
|      | 4,501,317 A                                       | 2/1985 Sokolowski                                                                                                                                                                                                                                                       | 9,616,493 B2    | 4/2017      | Tilak et al.        |                    |  |
|      | 4,524,819 A                                       | 6/1985 Yoshimura                                                                                                                                                                                                                                                        | 2007/0074846 A1 | 4/2007      | Sommerhofer et al.  |                    |  |
|      | 4,527,609 A *                                     | 7/1985 Nugent .....                                                                                                                                                                                                                                                     | 2009/0269239 A1 | 10/2009     | Nagakura et al.     |                    |  |
|      |                                                   | <i>B22D 11/04</i>                                                                                                                                                                                                                                                       | 2011/0209843 A2 | 9/2011      | Bes et al.          |                    |  |
|      |                                                   | 164/253                                                                                                                                                                                                                                                                 | 2011/0247456 A1 | 10/2011     | Rundquist et al.    |                    |  |
|      |                                                   |                                                                                                                                                                                                                                                                         | 2012/0148593 A1 | 6/2012      | Elson et al.        |                    |  |
|      |                                                   |                                                                                                                                                                                                                                                                         | 2012/0237395 A1 | 9/2012      | Jarry               |                    |  |
|      | FOREIGN PATENT DOCUMENTS                          |                                                                                                                                                                                                                                                                         |                 |             |                     |                    |  |
|      | 4,528,099 A                                       | 7/1985 Rieger et al.                                                                                                                                                                                                                                                    | CN              | 1059484 A   | 3/1992              |                    |  |
|      | 4,553,604 A                                       | 11/1985 Yaji et al.                                                                                                                                                                                                                                                     | CN              | 1064034     | 9/1992              |                    |  |
|      | 4,556,535 A                                       | 12/1985 Bowman et al.                                                                                                                                                                                                                                                   | CN              | 1611311     | 5/2005              |                    |  |
|      | 4,567,936 A                                       | 2/1986 Binczewski                                                                                                                                                                                                                                                       | CN              | 1925938     | 3/2007              |                    |  |
|      | 4,581,295 A                                       | 4/1986 DeLiso et al.                                                                                                                                                                                                                                                    | CN              | 1925938 A   | 3/2007              |                    |  |
|      | 4,582,118 A                                       | 4/1986 Jacoby et al.                                                                                                                                                                                                                                                    | CN              | 101428334   | 5/2009              |                    |  |
|      | 4,593,745 A                                       | 6/1986 Yu et al.                                                                                                                                                                                                                                                        | CN              | 101648265   | 2/2010              |                    |  |
|      | 4,597,432 A                                       | 7/1986 Collins et al.                                                                                                                                                                                                                                                   | CN              | 101712071   | 5/2010              |                    |  |
|      | 4,598,763 A                                       | 7/1986 Wagstaff et al.                                                                                                                                                                                                                                                  | CN              | 101712071 A | 5/2010              |                    |  |
|      | 4,607,679 A                                       | 8/1986 Tsai et al.                                                                                                                                                                                                                                                      | CN              | 101967588   | 2/2011              |                    |  |
|      | 4,610,295 A                                       | 9/1986 Jacoby et al.                                                                                                                                                                                                                                                    | CN              | 201892583   | 7/2011              |                    |  |
|      | 4,628,985 A                                       | 12/1986 Jacoby et al.                                                                                                                                                                                                                                                   | CN              | 102699302   | 10/2012             |                    |  |
|      | 4,640,497 A                                       | 2/1987 Heamion                                                                                                                                                                                                                                                          | CN              | 104470655   | 3/2017              |                    |  |
|      | 4,651,804 A                                       | 3/1987 Grimes et al.                                                                                                                                                                                                                                                    | CN              | 105008064   | 6/2017              |                    |  |
|      | 4,709,740 A                                       | 12/1987 Jacoby et al.                                                                                                                                                                                                                                                   | DE              | 4328045     | 2/1995              |                    |  |
|      | 4,709,747 A                                       | 12/1987 Yu et al.                                                                                                                                                                                                                                                       | EP              | 0090583     | 10/1983             |                    |  |
|      | 4,724,887 A                                       | 2/1988 Jacoby et al.                                                                                                                                                                                                                                                    | EP              | 0109170     | 5/1984              |                    |  |
|      | 4,761,266 A *                                     | 8/1988 Bruski .....                                                                                                                                                                                                                                                     | EP              | 0142341     | 5/1985              |                    |  |
|      |                                                   | <i>C22C 1/026</i>                                                                                                                                                                                                                                                       | 266/95          | 0150922     | 8/1985              |                    |  |
|      |                                                   |                                                                                                                                                                                                                                                                         |                 | 0183563     | 6/1986              |                    |  |
|      | 4,769,158 A                                       | 9/1988 Eckert                                                                                                                                                                                                                                                           | EP              | 0229211     | 7/1987              |                    |  |
|      | 4,770,697 A                                       | 9/1988 Zurecki                                                                                                                                                                                                                                                          | EP              | 0229218     | 7/1987              |                    |  |
|      | 4,773,470 A                                       | 9/1988 Libby et al.                                                                                                                                                                                                                                                     | EP              | 0281238     | 9/1988              |                    |  |
|      | 4,781,239 A                                       | 11/1988 Cans et al.                                                                                                                                                                                                                                                     | EP              | 0295008     | 12/1988             |                    |  |
|      | 4,809,866 A                                       | 3/1989 Greene et al.                                                                                                                                                                                                                                                    | EP              |             |                     |                    |  |

(56)

## References Cited

## FOREIGN PATENT DOCUMENTS

|    |               |         |
|----|---------------|---------|
| EP | 0364097       | 4/1990  |
| EP | 0402692       | 12/1990 |
| EP | 0497254       | 8/1992  |
| EP | 0726114       | 8/1996  |
| EP | 1045216       | 10/2000 |
| EP | 2664397       | 3/2016  |
| GB | 2281312       | 3/1995  |
| JP | S60127059     | 7/1985  |
| JP | 60180656      | 11/1985 |
| JP | 62176642      | 8/1987  |
| JP | S63118027     | 5/1988  |
| JP | 1233051       | 9/1989  |
| JP | 4313455       | 11/1992 |
| JP | 557400        | 3/1993  |
| JP | 8268745       | 10/1996 |
| JP | 2002089542    | 3/2002  |
| JP | 2006297100    | 11/2006 |
| JP | 2009150248    | 7/2009  |
| RU | 2048568       | 11/1995 |
| RU | 2261933       | 10/2005 |
| RU | 2377096       | 12/2009 |
| RU | 2381865       | 2/2010  |
| WO | WO-8702069    | 4/1987  |
| WO | WO-2010094852 | 8/2010  |
| WO | 2013173649    | 11/2013 |
| WO | WO-2014121297 | 8/2014  |

## OTHER PUBLICATIONS

Almex USA, Inc., "Non final office action", U.S. Appl. No. 14/401,458, (dated May 10, 2017).

Almex USA, Inc., "Office Action", JP Application No. 2015-512865, (dated Feb. 20, 2017).

Almex USA, Inc., "Office Action", JP Application No. 2015-512862, (dated Feb. 28, 2017).

Almex USA, Inc., "Third Office Action", CN Application No. 201380037685.0, (dated Feb. 16, 2017).

Almex USA, Inc., "European extended search report", EP Application No. 14198973.1, (dated May 7, 2015).

Almex USA, Inc., "International preliminary report on patentability", PCT/US2014/014735, (dated Jul. 10, 2015).

Almex USA, Inc., "International Preliminary Report on Patentability", PCT/US2014/014737, (dated Jul. 10, 2015).

Almex USA Inc., "International preliminary report on patentability", PCT/US2013/041459, (dated Nov. 27, 2014).

Almex USA, Inc., "International Preliminary Report on Patentability", PCT/US2013/041464, (dated Nov. 27, 2014).

Almex USA, Inc., "International Preliminary Report on Patentability", PCT/US2013/041457, (dated Nov. 27, 2014).

Almex USA, Inc., "Invitation to pay additional fees", PCT/US2014/066755, (dated Feb. 26, 2015).

Almex USA, Inc., "Office action with search report", CN Application No. 201480001852.0, (dated Sep. 1, 2016).

Almex USA, Inc., "Written Opinion", PCT/US2014/014735, (dated Feb. 20, 2015).

Almex USA, Inc., "Written Opinion", PCT/US2014/014737, (dated Feb. 20, 2015).

Anonymous, "Concise description of relevance", U.S. Appl. No. 14/546,681, (filed Feb. 17, 2016).

Anonymous, "Explanation of Relevance", PCT/US2014/066755, (Feb. 10, 2016).

Anonymous, "PCT third party observation", PCT/US2014/066755, (Feb. 10, 2016).

Anonymous, "Third party submission", U.S. Appl. No. 14/546,681, (filed Feb. 17, 2016).

"Semi-Continuous Casting Plant Produces Aluminium-Lithium Alloys", Met. Ind. News 3, (Sep. 1986), Abstract.

Almex USA, PCT Search Report and Written Opinion for PCT/US2014/014737 dated Jun. 17, 2014.

Almex USA, PCT Search Report and Written Opinion for PCT/US2014/014735 dated Jun. 17, 2014.

Almex USA, Search Report dated Nov. 18, 2013 for European App 13150674.3.

Almex USA, PCT Search Report & Written Opinion dated Nov. 27, 2013 for PCT/US2013/041464.

Almex USA, Inc., International search report and written opinion dated Dec. 2, 2013 for PCT/US2013/041459.

Almex USA, Inc., Non-Final Office Action dated Nov. 6, 2012 for U.S. Appl. No. 13/474,616.

Gorss, J. B., et al., "Design and operation experience with a coreless inductor furnace for melting aluminum", 12th ABB Conference on Induction Furnaces, Dortmund, Germany, (Apr. 17-18, 1991), pp. 301-313.

Heine, H. G., et al., "Coreless Induction Melting of Aluminum", Light Metal Age, (Feb. 1991), pp. 18-23.

Nair, C. G., et al., "Technology for Aluminium-Lithium Alloy Production—Ingot Casting Route", Science and Technology of Aluminium-Lithium Alloys, Bangalore, India, (Mar. 4-5, 1989), Abstract.

Ohara, K., et al., "Hot-tearing of Al—Li alloys in DC casting", 4th International Conference on Aluminum Alloys: Their Physical and Mechanical Properties, vol. II, (Sep. 11-16, 1994), Abstract.

Page, F. M., et al., "The Safety of Molten Aluminium-Lithium Alloys in the Presence of Coolants", Journal de Physique 48, Supplement No. 9, (Sep. 1987), C3-63-C3-73.

Almex USA, Inc., "European Search Report", EP Application No. 16182786.0, (dated Dec. 15, 2016).

Almex USA, Inc., "First Office Action", CN Application No. 201480007290.0, (dated Aug. 1, 2016).

Almex USA, Inc., "Final office action", JP Application No. 2015-512865 (dated Jul. 26, 2017).

Almex USA, Inc. "Non final office action", U.S. Appl. No. 14/546,681 (dated Jun. 23, 2017).

Almex USA, Inc. "Notice of Allowance", U.S. Appl. No. 14/401,813 (dated Jun. 9, 2017).

\* cited by examiner



**FIG. 2**

**FIG. 3**

## PROCESS AND APPARATUS FOR DIRECT CHILL CASTING

### CROSS-REFERENCE TO RELATED APPLICATION

This application is a non-provisional application claiming the benefit of International Patent Application No. PCT/US2013/041459, filed May 16, 2013, which claims the earlier filing date of co-pending U.S. patent application Ser. No. 13/474,614, filed May 17, 2012 and incorporated herein by reference.

### FIELD

Direct chill casting of aluminum lithium (Al—Li) alloys.

### BACKGROUND

Traditional (non-lithium containing) aluminum alloys have been semi-continuously cast in open bottomed molds since the invention of Direct Chill (“DC”) casting in the 1938 by the Aluminum Company of America (now Alcoa). Many modifications and alterations to the process have occurred since then, but the basic process and apparatus remain similar. Those skilled in the art of aluminum ingot casting will understand that new innovations improve the process, while maintaining its general functions.

U.S. Pat. No. 4,651,804 describes a more modern aluminum casting pit design. It has become standard practice to mount the metal melting furnace slightly above ground level with the casting mold at, or near to, ground level and the cast ingot is lowered into a water containing pit as the casting operation proceeds. Cooling water from the direct chill flows into the pit and is continuously removed there-from while leaving a permanent deep pool of water within the pit. This process remains in current use and, throughout the world, probably in excess of 5 million tons of aluminum and its alloys are produced annually by this method.

Unfortunately, there is inherent risk from a “bleed-out” or “run-out” using such systems. A “bleed-out” or “run-out” occurs where the aluminum ingot being cast is not properly solidified in the casting mold, and is allowed to leave the mold unexpectedly and prematurely while in a liquid state. Molten aluminum in contact with water during a “bleed-out” or “run-out” can cause an explosion from (1) conversion of water to steam from the thermal mass of the aluminum heating the water to >212° F. or (2) the chemical reaction of the molten metal with the water resulting in release of energy causing an explosive chemical reaction.

There have been many explosions throughout the world when “bleed-outs” “run-outs” have occurred in which molten metal escaped from the sides of the ingot emerging from the mold and/or from the confines of the mold, using this process. In consequence, considerable experimental work has been carried out to establish the safest possible conditions for DC casting. Among the earliest and perhaps the best known work was undertaken by G. Long of the Aluminum Company of America (“Metal Progress” May 1957 pages 107 to 112) (hereinafter referred to as “Long”) that was followed by further investigations and the establishment of industry “codes of practice” designed to minimize the risk of explosion. These codes are generally followed by foundries throughout the world. The codes are broadly based upon Long’s work and usually require that: (1) the depth of water permanently maintained in the pit should be at least three feet; (2) the level of water within the pit should be at least

10 feet below the mold; and (3) the casting machine and pit surfaces should be clean, rust free and coated with proven organic material.

In his experiments, Long found that with a pool of water in the pit having a depth of two inches or less, very violent explosions did not occur. However, instead, lesser explosions took place sufficient to discharge molten metal from the pit and distribute this molten metal in a hazardous manner externally of the pit. Accordingly the codes of practice, as stated above, require that a pool of water having a depth of at least three feet is permanently maintained in the pit. Long had drawn the conclusion that certain requirements must be met if an aluminum/water explosion is to occur. Among these was that a triggering action of some kind must take place on the bottom surface of the pit when it is covered by molten metal and he suggested that this trigger is a minor explosion due to the sudden conversion to steam of a very thin layer of water trapped below the incoming metal. When grease, oil or paint is on the pit bottom an explosion is prevented because the thin layer of water necessary for a triggering explosion is not trapped beneath the molten metal in the same manner as with an uncoated surface.

In practice, the recommended depth of at least three feet of water is generally employed for vertical DC casting and in some foundries (notably in continental European countries) the water level is brought very close to the underside of the mold in contrast to recommendation (2) above. Thus the aluminum industry, casting by the DC method, has opted for the safety of a deep pool of water permanently maintained in the pit. It must be emphasized that the codes of practice are based upon empirical results; what actually happens in various kinds of molten metal/water explosions is imperfectly understood. However, attention to the codes of practice has ensured the virtual certainty of avoiding accidents in the event of “run-outs” with aluminum alloys.

In the last several years, there has been growing interest in light metal alloys containing lithium. Lithium makes the molten alloys more reactive. In the above mentioned article in “Metal Progress”, Long refers to previous work by H. M. Higgins who had reported on aluminum/water reactions for a number of alloys including Al—Li and concluded that “When the molten metals were dispersed in water in any way Al—Li alloy underwent a violent reaction.” It has also been announced by the Aluminum Association Inc. (of America) that there are particular hazards when casting such alloys by the DC process. The Aluminum Company of America has published video recordings of tests that demonstrate that such alloys can explode with great violence when mixed with water.

U.S. Pat. No. 4,651,804 teaches the use of the aforementioned casting pit, but with the provision of removing the water from the bottom of the cast pit such that no buildup of a pool of water in the pit occurs. This arrangement is their preferred methodology for casting Al—Li alloys. European Patent No. 0-150-922 describes a sloped pit bottom (preferably three percent to eight percent inclination gradient of the pit bottom) with accompanying off-set water collection reservoir, water pumps, and associated water level sensors to make sure water cannot collect in the cast pit, thus reducing the incidence of explosions from water and the Al—Li alloy having intimate contact. The ability to continuously remove the ingot coolant water from the pit such that a build-up of water cannot occur is critical to the success of the patent’s teachings.

Other work has also demonstrated that the explosive forces associated with adding lithium to aluminum alloys can increase the nature of the explosive energy several times

than for aluminum alloys without lithium. When molten aluminum alloys containing lithium come into contact with water, there is the rapid evolution of hydrogen, as the water dissociates to Li—OH and hydrogen ion (H<sup>+</sup>). U.S. Pat. No. 5,212,343 teaches the addition of aluminum, lithium (and other elements as well) with water to initiate explosive reactions. The exothermic reaction of these elements (particularly aluminum and lithium) in water produces large amounts of hydrogen gas, typically 14 cubic centimeters of hydrogen gas per one gram of aluminum—3% lithium alloy. Experimental verifications of this data can be found in the research carried out under U.S. Department of Energy funded research contract number #DE-AC09-89SR18035. Note that Claim 1 of the U.S. Pat. No. 5,212,343 patent claims the method to perform this intense interaction for producing a water explosion via the exothermic reaction. This patent describes a process wherein the addition of elements such as lithium results in a high energy of reaction per unit volume of materials. As described in U.S. Pat. Nos. 5,212,343 and 5,404,813, the addition of lithium (or some other chemically active element) promotes an explosion. These patents teach a process where an explosive reaction is a desirable outcome. These patents reinforce the explosiveness of the addition of lithium to the “bleed-out” or “run-out”, as compared to aluminum alloys without lithium.

Referring again to the U.S. Pat. No. 4,651,804, the two occurrences that result in explosions for conventional (non-lithium bearing) aluminum alloys are (1) conversion of water to steam and (2) the chemical reaction of molten aluminum and water. The addition of lithium to the aluminum alloy produces a third, even more acute explosive force, the exothermic reaction of water and the molten aluminum-lithium “bleed-out” or “run-out” producing hydrogen gas. Any time the molten Al—Li alloy comes into contact with water, the reaction will occur. Even when casting with minimum water levels in the casting pit, the water comes into contact with the molten metal during a “bleed-out” or “run-out”. This cannot be avoided, only reduced, since both components (water and molten metal) of the exothermic reaction will be present in the casting pit. Reducing the amount of water-to-aluminum contact will eliminate the first two explosive conditions, but the presence of lithium in the aluminum alloy will result in hydrogen evolution. If hydrogen gas concentrations are allowed to reach a critical mass and/or volume in the casting pit, explosions are likely to occur. The volume concentration of hydrogen gas required for triggering an explosion has been researched to be at a threshold level of 5% of volume of the total volume of the mixture of gases in a unit space. U.S. Pat. No. 4,188,884 describes making an underwater torpedo warhead, and recites page 4, column 2, line 33 referring to the drawings that a filler 32 of a material which is highly reactive with water, such as lithium is added. At column 1, line 25 of this same patent it is stated that large amounts of hydrogen gas are released by this reaction with water, producing a gas bubble with explosive suddenness.

U.S. Pat. No. 5,212,343 describes making an explosive reaction by mixing water with a number of elements and combinations, including Al and Li to produce large volumes of hydrogen containing gas. On page 7, column 3, it states “the reactive mixture is chosen that, upon reaction and contact with water, a large volume of hydrogen is produced from a relatively small volume of reactive mixture.” Same paragraph, lines 39 and 40 identify aluminum and lithium. On page 8, column 5, lines 21-23 show aluminum in combination with lithium. On page 11 of this same patent, column 11, lines 28-30 refer to a hydrogen gas explosion.

In another method of conducting DC casting, patents have been issued related to casting Al—Li alloys using an ingot coolant other than water to provide ingot cooling without the water-lithium reaction from a “bleed-out” or “run-out”. U.S. Pat. No. 4,593,745 describes using a halogenated hydrocarbon or halogenated alcohol as ingot coolant. U.S. Pat. Nos. 4,610,295; 4,709,740, and 4,724,887 describe the use of ethylene glycol as the ingot coolant. For this to work, the halogenated hydrocarbon (typically ethylene glycol) must be free of water and water vapor. This is a solution to the explosion hazard, but introduces strong fire hazard and is costly to implement and maintain. A fire suppression system will be required within the casting pit to contain potential glycol fires. To implement a glycol based ingot coolant system including a glycol handling system, a thermal oxidizer to de-hydrate the glycol, and the casting pit fire protection system generally costs on the order of \$5 to \$8 million dollars (in today’s dollars). Casting with 100% glycol as a coolant also brings in another issue. The cooling capability of glycol or other halogenated hydrocarbons is different than that for water, and different casting practices as well as casting tooling are required to utilize this type of technology. Another disadvantage affiliated with using glycol as a straight coolant is that because glycol has a lower heat conductivity and surface heat transfer coefficient than water, the microstructure of the metal cast with 100% glycol as a coolant has coarser undesirable metallurgical constituents and exhibits higher amount of centerline shrinkage porosity in the cast product. Absence of finer microstructure and simultaneous presence of higher concentration of shrinkage porosity has a deleterious effect on the properties of the end products manufactured from such initial stock.

In yet another example of an attempt to reduce the explosion hazard in the casting of Al—Li alloys, U.S. Pat. No. 4,237,961, suggests removing water from the ingot during DC casting. In European Patent No. 0-183-563, a device is described for collecting the “break-out” or “run-out” molten metal during direct chill casting of aluminum alloys. Collecting the “break-out” or “run-out” molten metal would concentrate this mass of molten metal. This teaching cannot be used for Al—Li casting since it would create an artificial explosion condition where removal of the water would result in a pooling of the water as it is being collected for removal. During a “bleed-out” or “run-out” of the molten metal, the “bleed-out” material would also be concentrated in the pooled water area. As taught in U.S. Pat. No. 5,212,343, this would be a preferred way to create a reactive water/Al—Li explosion.

Thus, numerous solutions have been proposed in the prior art for diminishing or minimizing the potential for explosions in the casting of Al—Li alloys. While each of these proposed solutions has provided an additional safeguard in such operations, none has proven to be entirely safe or commercially cost effective.

Thus, there remains a need for safer, less maintenance prone and more cost effective apparatus and processes for casting Al—Li alloys that will simultaneously produce a higher quality of the cast product.

#### DESCRIPTION OF THE DRAWINGS

FIG. 1 is a simplified cross sectional side view of an embodiment of a direct chill casting pit.

FIG. 2 is a process flow diagram of an embodiment of a process addressing a “bleed-out” or a “run-out” in a casting operation.

FIG. 3 is a process flow diagram of another embodiment of a process addressing a “bleed-out” or a “run-out” in a casting operation.

## DETAILED DESCRIPTION

An apparatus and method for casting Al—Li alloys is described. A concern with prior art teachings is that water and the Al—Li molten metal “bleed-out” or “run-out” materials come together and release hydrogen during an exothermic reaction. Even with sloped pit bottoms, minimum water levels, etc., the water and “bleed-out” or “run-out” molten metal may still come into intimate contact, enabling the reaction to occur. Casting without water, using another liquid such as those described in prior art patents affects castability, quality of the cast product, is costly to implement and maintain, as well as poses environmental concerns and fire hazards.

The instantly described apparatus and method improve the safety of DC casting of Al—Li alloys by minimizing or eliminating ingredients that must be present for an explosion to occur. It is understood that water (or water vapor or steam) in the presence of the molten Al—Li alloy will produce hydrogen gas. A representative chemical reaction equation is believed to be:



Hydrogen gas has a density significantly less than a density of air. Hydrogen gas that evolves during the chemical reaction, being lighter than air, tends to gravitate upward, toward the top of a cast pit, just below the casting mold and mold support structures at the top of the casting pit. This typically enclosed area allows the hydrogen gas to collect and become concentrated enough to create an explosive atmosphere. Heat, a spark, or other ignition source can trigger the explosion of the hydrogen ‘plume’ of the as-concentrated gas.

It is understood that the molten “bleed-out” or “run-out” material when combined with the ingot cooling water that is used in a DC process (as practiced by those skilled in the art of aluminum ingot casting) will create steam and water vapor. The water vapor and steam are accelerants for the reaction that produces the hydrogen gas. Removal of this steam and water vapor by a steam removal system will remove the ability of the water to combine with Al—Li creating Li—OH, and the expulsion of H<sub>2</sub>. The instantly described apparatus and method minimizes the potential for the presence of water and steam vapor in the casting pit by, in one embodiment, placing steam exhaust ports about the inner periphery of the casting pit, and rapidly activating the vents upon the detection of an occurrence of a “bleed-out”.

According to one embodiment, the exhaust ports are located in several areas within the casting pit, e.g., from about 0.3 meters to about 0.5 meters below the casting mold, in an intermediate area from about 1.5 meters to about 2.0 meters from the casting mold, and at the bottom of the cast pit. For reference, and as shown in the accompanying drawings described in greater detail below, a casting mold is typically placed at a top of a casting pit, from floor level to as much as one meter above floor level. The horizontal and vertical areas around the casting mold below the mold table are generally closed-in with a pit skirt and a Lexan glass encasement except for the provision to bring in and ventilate outside air for dilution purpose, such that the gasses contained within the pit are introduced and exhausted according to a prescribed manner.

In another embodiment, an inert gas is introduced into the casting pit interior space to minimize or eliminate the coalition of hydrogen gas into a critical mass. In this case, the inert gas is a gas that has a density less than a density of air and that will tend to occupy the same space just below the top of the casting pit that hydrogen gas would typically inhabit. Helium gas is one such example of suitable inert gas with a density less than a density of air.

The use of argon has been described in numerous technical reports as a cover gas for protecting Al—Li alloys from ambient atmosphere to prevent their reaction with air. Even though argon is completely inert, it has a density greater than a density of air and will not provide the inerting of the casting pit upper interior unless a strong upward draft is maintained. Compared to air as a reference (1.3 grams/liter), argon has density on the order of 1.8 grams/liter and would tend to settle to the bottom of a cast pit, providing no desirable hydrogen displacement protection within the critical top area of the casting pit. Helium, on the other hand, is nonflammable and has a low density of 0.2 grams per liter and will not support combustion. By exchanging air for a lower density of inert gas inside a casting pit, the dangerous atmosphere in the casting pit may be diluted to a level where an explosion cannot be supported. Also, while this exchange is occurring, water vapor and steam are also removed from the casting pit. In one embodiment, during steady state casting and when non-emergency condition pertaining to a ‘bleed-out’ is not being experienced, the water vapor and steam are removed from the inert gas in an external process, while the ‘clean’ inert gas can be re-circulated back through the casting pit.

Referring now to the accompanying drawings, FIG. 1 shows a cross-section of an embodiment of a DC casting system. DC system 5 includes casting pit 16 that is typically formed into the ground. Disposed within casting pit 16 is casting cylinder 15 that may be raised and lowered, for example, with a hydraulic power unit (not shown). Attached to a superior or top portion of casting cylinder 15 is platen 18 that is raised and lowered with casting cylinder 15. Above or superior to platen 18 in this view is stationary casting mold 12. Molten metal (e.g., Al—Li alloy) is introduced into mold 12. Casting mold 12, in one embodiment, includes, coolant inlets to allow coolant (e.g., water) to flow onto a surface of an emerging ingot providing a direct chill and solidification of the metal. Surrounding casting mold 12 is casting table 31. As shown in FIG. 1, in one embodiment, a gasket or seal 29 fabricated from, for example, a high temperature resistant silica material is located between the structure of mold 12 and table 31. Gasket 29 inhibits steam or any other atmosphere from below mold table 31 to reach above the mold table and thereby inhibits the pollution of the air in which casting crewmen operate and breathe.

In the embodiment shown in FIG. 1, system 5 includes molten metal detector 10 positioned just below mold 12 to detect a bleed-out or run-out. Molten metal detector 10 may be, for example, an infrared detector of the type described in U.S. Pat. No. 6,279,645, a “break out detector” as described in U.S. Pat. No. 7,296,613 or any other suitable device that can detect the presence of a “bleed-out”.

In the embodiment shown in FIG. 1, system 5 also includes exhaust system 19. In one embodiment, exhaust system 19 includes, in this embodiment, exhaust ports 20A, 20A', 20B, 20B', 20C and 20C' positioned in casting pit 16. The exhaust ports are positioned to maximize the removal of generated gases including ignition sources (e.g., H<sub>2</sub>(g)) and reactants (e.g., water vapor or steam) from the inner cavity of the casting pit. In one embodiment, exhaust ports 20A,

20A' are positioned about 0.3 meters to about 0.5 meters below mold 12; exhaust ports 20B, 20B' are positioned about 1.5 meters to about 2.0 meters below the mold 12; and exhaust ports 20C, 20C' are positioned at a base of casting pit 16 where bleed-out metal is caught and contained. The exhaust ports are shown in pairs at each level. It is appreciated that, in an embodiment where there are arrays of exhaust ports at different levels such as in FIG. 1, there may be more than two exhaust ports at each level. For example, in another embodiment, there may be three or four exhaust ports at each level. In another embodiment, there may be less than two (e.g., one at each level). Exhaust system 19 also includes remote exhaust vent 22 that is remote from casting mold 12 (e.g., about 20 to 30 meters away from mold 12) to allow exit of exhausted gases from the system. Exhaust ports 20A, 20A', 20B, 20B', 20C, 20C' are connected to exhaust vent 22 through ducting (e.g., galvanized steel or stainless steel ducting). In one embodiment, exhaust system 19 further includes an array of exhaust fans to direct exhaust gases to exhaust vent 22.

FIG. 1 further shows gas introduction system 24 including, in this embodiment, inert gas introduction ports (e.g., inert gas introduction ports 26A, 26A', 26B, 26B', 26C and 26C') disposed around the casting pit and connected to an inert gas source or sources 27. In one embodiment, concurrent to positions of each of ports 26B and 26B', and 26C and 26C', there are positioned excess air introduction ports to assure additional in-transit dilution of the evolved hydrogen gas. The positioning of gas introduction ports is selected to provide a flood of inert gas to immediately replace the gases and steam within the pit, via a gas introduction system 24 that introduces inert gas as and when needed (especially upon the detection of a bleed-out) through inert gas introduction ports 26 into casting pit 16 within a predetermined time (e.g., about a maximum of 30 seconds) of the detection of a “bleed-out” condition. FIG. 1 shows gas introduction ports 26A and 26A' positioned near a top portion of casting pit 16; gas introduction ports 26B and 26B' positioned at an intermediate portion of casting pit 16; and gas introduction ports 26C and 26C' positioned at a bottom portion of casting pit 16. Pressure regulators may be associated with each gas introduction port to control the introduction of an inert gas. The gas introduction ports are shown in pairs at each level. It is appreciated that, in an embodiment, where there are arrays of gas introduction ports at each level, there may be more than two gas introduction ports at each level. For example, in another embodiment, there may be three or four gas introduction ports at each level. In another embodiment, there may be less than two (e.g., one) at each level.

As shown in FIG. 1, in one embodiment, the inert gas introduced through gas introduction ports 26A and 26A' at top 14 of casting pit 16 should impinge on the solidified, semi-solid and liquid aluminum lithium alloy below mold 12, and inert gas flow rates in this area are, in one embodiment, at least substantially equal to a volumetric flow rate of a coolant prior to detecting the presence of a “bleed-out” or a “run-out”. In embodiments where there are gas introduction ports at different levels of a casting pit, flow rates through such gas introduction ports may be the same as a flow rate through the gas introduction ports at top 14 of casting pit 16 or may be different (e.g., less than a flow rate through the gas introduction ports at top 14 of casting pit 16).

The replacement inert gas introduced through the gas introduction ports is removed from casting pit 16 by an upper exhaust system 28 which is kept activated at lower volume on continuous basis but the volume flow rate is

enhanced immediately upon detection of a “bleed-out” and directs inert gas removed from the casting pit to the exhaust vent 22. In one embodiment, prior to the detection of bleed-out, the atmosphere in the upper portion of the pit may be continuously circulated through atmosphere purification system 30 of, for example, moisture stripping columns and steam desiccants thus keeping the atmosphere in the upper region of the pit reasonably inert. The removed gas while being circulated is passed through atmosphere purification system 30 and any water vapor is removed to purify the upper pit atmosphere containing inert gas. The purified inert gas may then be re-circulated to inert gas injection system 24 via a suitable pump 32. When this embodiment is employed, inert gas curtains are maintained, between the ports 20A and 26A and similarly between the ports 20A' and 26A' to minimize the escape of the precious inert gas of the upper region of the casting pit through the pit ventilation and exhaust system.

The number and exact location of exhaust ports 20A, 20A', 20B, 20B', 20C, 20C' and inert gas introduction ports 26A, 26A', 26B, 26B', 26C, 26C' will be a function of the size and configuration of the particular casting pit being operated and these are calculated by the skilled artisan practicing DC casting in association with those expert at recirculation of air and gases. It is most desirable to provide the three sets (e.g., three pairs) of exhaust ports and inert gas introduction ports as shown FIG. 1. Depending on the nature and the weight of the product being cast, a somewhat less complicated and less expensive but equally effective apparatus can be obtained using a single array of exhaust ports and inert gas introduction ports about the periphery of the top of casting pit 16.

In one embodiment, each of a movement of platen 18/casting cylinder 15, a molten metal supply inlet to mold 12 and a water inlet to the mold are controlled by controller 35. Molten metal detector 10 is also connected to controller 35. Controller 35 contains machine-readable program instructions as a form of non-transitory tangible media. In one embodiment, the program instructions are illustrated in the method of FIG. 2. Referring to FIG. 2 and method 100, first an Al—Li molten metal “bleed-out” or “run-out” is detected by molten metal detector 10 (block 110). In response to a signal from molten metal detector 10 to controller 35 of an Al—Li molten metal “bleed-out” or “run-out”, the machine readable instructions cause movement of platen 18 and molten metal inlet supply (not shown) to stop (blocks 120, 130), coolant flow (not shown) into mold 12 to stop and/or be diverted (block 140), and higher volume exhaust system 19 to be activated simultaneously or within about 15 seconds and in another embodiment, within about 10 seconds, to divert the water vapor containing exhaust gases and/or water vapor away from the casting pit via exhaust ports 20A, 20A', 20B, 20B', 20C and 20C' to exhaust vent 22 (block 150). At the same time or shortly thereafter (e.g., within about 10 seconds to within about 30 seconds), the machine readable instructions further activate gas introduction system and an inert gas having a density less than a density of air, such as helium, is introduced through gas introduction ports 26A, 26A', 26B, 26B', 26C and 26C' (block 160). The introduced inert gas is subsequently collected via the exhaust system and may then be purified (block 170). It is to be noted that those skilled in the art of melting and direct chill casting of aluminum alloys except the melting and casting of aluminum-lithium alloys may be tempted to use nitrogen gas in place of helium because of the general industrial knowledge that nitrogen is also an ‘inert’ gas. However, for the reason of maintaining

process safety, it is mentioned herein that nitrogen is really not an inert gas when it comes to interacting with liquid aluminum-lithium alloys. Nitrogen does react with the alloy and produces ammonia which in turns reacts with water and brings in additional reactions of dangerous consequences, and hence its use should be completely avoided. The same holds true for another presumably inert gas carbon dioxide. Its use should be avoided in any application where there is a finite chance of molten aluminum lithium alloy to get in touch with carbon dioxide.

A significant benefit obtained through the use of an inert gas that is lighter than air is that the residual gases will not settle into the casting pit, resulting in an unsafe environment in the pit itself. There have been numerous instances of heavier than air gases residing in confined spaces resulting in death from asphyxiation. It would be expected that the air within the casting pit will be monitored for confined space entry, but no process gas related issues are created.

FIG. 3 shows another embodiment of a method. Referring to FIG. 3 and method 200 and using the DC casting system of FIG. 1, first a molten metal “bleed-out” or “run-out” is detected by molten metal detector 10 (block 210). In response to a signal between molten metal detector 10 and controller 35 of a “bleed-out” or “run-out”, coolant flow into mold 12 is reduced (block 240); metal supply into the mold is stopped (block 230); and a movement of platen 18 is reduced (block 220). With regard to a reduction of a coolant flow and reduction of platen movement, such reduction may be a complete reduction (stop or halt) or a partial reduction. For example, a coolant flow rate may be reduced to a rate that is greater than a flow rate of zero, but less than a predetermined flow rate selected to flow onto an emerging ingot providing a direct chill and solidification of the metal. In one embodiment, the flow rate is reduced to a rate that is acceptably safe (e.g., a few liters per minute or less) given the additional measures that are implemented to address the “bleed-out” or “run-out”. Similarly, platen 18 can continue to move through casting pit 16 at a rate that is acceptably safe but that is reduced from a predetermined selected rate to cast metal. Finally, in one embodiment, a reduction in coolant flow and platen movement need not be related in the sense that they are either both reduced to complete cessation or to a rate greater than complete cessation. In other words, in one embodiment, a coolant flow rate may be stopped or halted (i.e., reduced to a flow rate of zero) following a detection of a “bleed-out” and a platen movement may be reduced to a rate tending to halting or stopping, but not halted or stopped, i.e., a rate of movement greater than zero. In another embodiment, a movement of platen 18 may be halted or stopped (i.e., reduced to a rate of zero) while a rate of coolant flow reduced to rate tending to halting or stopping, but not halted or stopped, i.e., a rate of flow greater than zero. In yet another embodiment, coolant flow and movement of platen 18 are both halted or stopped.

In another embodiment, upon detection of a “bleed-out” or “run-out”, machine readable instructions implementing the method of FIG. 3 direct an evacuation of exhaust gases and/or water vapor from casting pit 16 (block 250); introduce inert gas into the pit (block 260); and optionally collect and/or purify inert gas removed from the pit (block 270) similar to the method described above with respect to FIG. 2.

In the casting system described above with reference to FIG. 1, system 5 included molten metal detector 10 configured to detect a “bleed-out” or a “run-out”. Embodiments of methods described with reference to FIG. 2 and FIG. 3 included embodiments where a detection device, such as

molten metal detector 10, is communicatively linked with a controller (e.g., controller 35 in system 5 of FIG. 1) such that a molten metal detector 10 detects a “bleed-out” or a “run-out” and communicates the condition to controller 35. 5 In another embodiment, with or without molten metal detector 10 or a link between detector 10 and controller 35, a “bleed-out” and “run-out” may be detected. One way is by an operator operating system 5 and visually observing a “bleed-out” or “run-out”. In such instance, the operator may 10 communicate with controller 35 to implement actions by controller 35 to minimize effects of a “bleed-out” or a “run-out” (e.g., exhausting generated gas from the casting pit, introducing an inert gas into the casting pit, stopping flow of metal, reducing or stopping flow of coolant, reducing 15 or stopping movement of platen, etc.). Such communication may be, for example, pressing a key or keys on a keypad associated with controller 35.

The process and apparatus described herein provide a unique method to adequately contain Al—Li “bleed-outs” or 20 “run-outs” such that a commercial process can be operated successfully without utilization of extraneous process methods, such as casting using a halogenated liquid like ethylene glycol that render the process not optimal for cast metal quality, a process less stable for casting, and at the same time 25 a process which is uneconomical and flammable. As anyone skilled in the art of ingot casting will understand, it must be stated that in any DC process, “bleed-outs” and “run-outs” will occur. The incidence will generally be very low, but during the normal operation of mechanical equipment, 30 something will occur outside the proper operating range and the process will not perform as expected. The implementation of the described apparatus and process and use of this apparatus will minimize water-to-molten metal hydrogen explosions from “bleed-outs” or “run-outs” while casting 35 Al—Li alloys that result in casualties and property damage.

There has thus been described a commercially useful method and apparatus for minimizing the potential for explosions in the direct chill casting of Al—Li alloys. It is appreciated that though described for Al—Li alloys, the 40 method and apparatus can be used in the casting of other metals and alloys.

As the invention has been described, it will be apparent to those skilled in the art that the same may be varied in many ways without departing from the spirit and scope of the 45 invention. Any and all such modifications are intended to be included within the scope of the appended claims.

#### What is claimed is:

1. A process in direct chill casting wherein molten metal is introduced into a casting mold and cooled by impingement of a liquid coolant on solidifying metal in a casting pit including a movable platen and an occurrence of a bleed-out or run-out is detected, the process comprising:  
55 exhausting generated gas from the casting pit;  
while exhausting generated gas, introducing an inert gas into the casting pit, the inert gas having a density less than a density of air; and  
reducing any flow of the liquid coolant.
2. The process of claim 1, wherein the inert gas is helium.
3. The process of claim 1, wherein exhausting generated gas from the casting pit comprises exhausting by an array of 60 exhaust ports about at least a periphery of a top portion of the casting pit.
4. The process of claim 3, wherein exhausting generated gas further comprises exhausting by arrays of exhaust ports about an intermediate portion and a bottom portion of the casting pit.

## 11

5. The process of claim 1, wherein introducing an inert gas comprises introducing an inert gas through an array of gas introduction ports about a periphery of at least a top portion of the casting pit.

6. The process of claim 1, wherein introducing an inert gas comprises introducing an inert gas through arrays of gas introduction ports about a periphery of a top portion, an intermediate portion and a bottom portion of the casting pit.

7. The process of claim 1, wherein exhausting of generated gas comprises exhausting at a volume flow rate that is enhanced relative to a volume flow rate prior to the occurrence of a bleed-out or a run-out.

8. The process of claim 7, wherein enhanced exhausting of generated gas commences at a maximum of 15 seconds after detection of a bleed-out.

9. The process of claim 1, wherein introducing an inert gas in to the pit commences within a maximum of about 15 seconds after detection of a bleed-out.

10. The process of claim 1, wherein exhausting of generated gas comprises exhausting to a location at least 20 meters from the casting mold.

11. The process of claim 1, wherein introducing an inert gas comprises impinging the inert gas upon a metal being cast at a flow rate substantially equal to a volumetric flow rate selected for a liquid coolant prior to the occurrence of the bleed-out or run-out.

12. The process of claim 1, further comprising purifying inert gas via a gas purification system.

13. The process of claim 1, wherein after detecting the bleed-out or run-out, the process further comprising:

stopping introduction of a metal into the casting mold.

14. The process of claim 1, wherein reducing any flow of the liquid coolant comprises reducing any flow of coolant to a flow rate of zero.

15. The process of claim 1, wherein reducing any flow of the liquid coolant comprises reducing the flow to a rate less than flow rate selected to provide a direct chill and solidification of the metal.

16. The process of claim 1, further comprising:

reducing any movement of the platen.

17. The process of claim 16, wherein reducing any movement of the platen comprises reducing any movement to a rate of zero.

18. The process of claim 16, wherein reducing any movement of the platen comprises reducing the rate from a rate selected to cast metal.

19. The process of claim 1 further comprising:

stopping any flow of molten metal and reducing any movement of the platen,

wherein exhausting generated gas from the casting pit comprises exhausting at an enhanced flow volume rate

## 12

relative to a volume flow rate prior to the occurrence of a bleed-out or run-out by using an exhausting mechanism.

20. The process of claim 19, wherein the inert gas is helium.

21. The process of claim 19, wherein the casting pit comprises a top portion, an intermediate and a bottom portion and introducing an inert gas comprises introducing an inert gas through an array of gas introduction ports about a periphery of at least a top portion of the casting pit.

22. The process of claim 19, wherein introducing an inert gas comprises introducing an inert gas through arrays of gas introduction ports about a periphery of a top portion, an intermediate portion and a bottom portion of the casting pit.

23. The process of claim 19, wherein introducing an inert gas in to the pit commences within a maximum of about 15 seconds after detection of a bleed-out.

24. The process of claim 19, wherein exhausting of generated gas comprises exhausting to a location at least 20 meters from the casting mold.

25. The process of claim 19, wherein introducing an inert gas comprises impinging upon a solid, semi-solid or liquid metal portion of an ingot being cast at a flow rate substantially equal to a volumetric flow rate selected for a coolant prior to detecting a bleed-out or run-out.

26. The process of claim 19 further comprising reducing a flow of liquid coolant to a flow rate of zero.

27. The process of claim 19, wherein the molten metal comprises an aluminum lithium alloy.

28. The process of claim 1, wherein the casting pit comprises a top portion, an intermediate and a bottom portion and exhausting generated gas from the casting pit comprises exhausting by an array of exhaust ports about at least a periphery of the top portion of the casting pit, and the method further comprises stopping an introduction of molten metal into the casting mold.

29. The process of claim 1, wherein the casting pit comprises a top portion, an intermediate and a bottom portion and exhausting generated gas further comprises exhausting by arrays of exhaust ports about an intermediate portion and a bottom portion of the casting pit, and the method further comprises stopping a movement of the platen.

30. The process of claim 1, further comprising collecting the inert gas exhausted from the casting pit and purifying the collected gas via a gas purification system.

31. The process of claim 1 further comprising:

reducing any movement of the platen to a rate of zero; and stopping an introduction of molten metal into the casting mold.

32. The process of claim 1, wherein the molten metal comprises an aluminum lithium alloy.

\* \* \* \* \*